

# UNITED STATES PATENT OFFICE.

LAWRENCE E. BARRINGER AND FRANK C. ZAPF, OF SCHENECTADY, NEW YORK,  
ASSIGNORS TO GENERAL ELECTRIC COMPANY, A CORPORATION OF NEW YORK.

## INSULATING COMPOUND.

1,093,967.

Specification of Letters Patent. Patented Apr. 21, 1914.

No Drawing.

Application filed September 12, 1911. Serial No. 648,993.

*To all whom it may concern:*

Be it known that we, LAWRENCE E. BARRINGER and FRANK C. ZAPF, citizens of the United States, residing at Schenectady, county of Schenectady, State of New York, have invented certain new and useful Improvements in Insulating Compounds, of which the following is a specification.

This invention relates to insulating materials for electrical purposes and has for its object the provision of a material of this character having a high insulating value which does not diminish with a rise of temperature and which deteriorates very slowly with age.

More specifically, our invention relates to insulating materials in the nature of varnishes intended to be applied in a liquid form to a body to be insulated.

One of the uses to which insulating varnishes have been commonly put is for the purpose of making an insulating covering composed of a plurality of layers or coats of the varnish successively applied and permitted to harden before the next succeeding coat is applied. Fabrics thus treated are commonly used in the electrical arts as insulating coverings for coils and the like. Insulation of this character is disclosed in Emmet Patents 666,003 and 666,004. The particular varnish referred to in said patents, which has been commonly used for several years, is a varnish having a large percentage of an oxidizing oil, and about 80 parts to 20 parts of rosin. Linseed oil has been most commonly employed as the oxidizing oil. We have found that China wood oil has distinct advantages over linseed oil for this purpose and that when this is used the percentage of the oxidizing oil may be reduced with advantage.

One of the most remarkable properties of China wood oil is its resistance to aging. It is a well known fact that when linseed oil varnishes are exposed to heat for any great length of time, the film becomes brittle. China wood oil is not thus affected and in fact may be exposed to a temperature of 100° C. for a long time, after which the film is elastic and tough. This exposure to a temperature of 100° C. has been carried on for two hundred hours without affecting the film, while the same test with linseed oil varnish causes the film to become brittle and weak. With China wood oil it is un-

necessary to use any of the drying agents used in linseed oil varnishes. It is the presence of these driers which tends to make them short-lived, aside from the oxidizing of the linseed oil itself. In China wood oil, since no driers are used, there are no harmful influences exerted from this source, and it has also been noticed that China wood oil apparently completely oxidizes less rapidly under the same conditions than linseed oil.

Instead of using China wood oil alone, we have found that a very good insulating varnish is produced by the addition of a certain amount of rubbery pitch, such as cotton stearin pitch, which gives a great amount of elasticity to the varnish. We find, however, that the pitch has a tendency to remain permanently viscous, giving a varnish which remains somewhat "tacky" or sticky, and to overcome this objection, as well as to increase the disruptive strength, we add a certain amount of asphalt. The asphalt and pitch together impart to the varnish a very high insulating resistance, very much higher than where oil alone is used or where the base consists of a gum such as rosin or copal. The China wood oil gives the varnish a greater amount of flexibility, toughness and a longer life than can be secured with linseed oil. In some cases, as for instance where the varnish is to be used for coating cloth, paper and the like, a certain amount of a mineral oil, such as cylinder oil, may be used. This causes the varnish to flow more easily and also increases the life and elasticity of the varnish. The addition of oil of this character has also the advantage of making the varnish self healing.

In the specific embodiment of our invention, therefore, we first make a base by melting together the pitch and asphalt. After these become thoroughly mixed China wood oil is added and, if desired, cylinder oil. The pitch which we have found very suitable for our purpose is a rubbery cotton stearin pitch, although other pitches of this character may be used. We have also found that a certain asphalt, known as gilsonite, serves our purpose very well, although any good hard asphalt may be used. While these materials may be combined in various proportions to produce insulating varnish, we have found the following proportions to

give excellent results: 25 per cent. China wood oil, 15 per cent. cylinder oil, 30 per cent. pitch, 30 per cent. asphalt. In some cases where it is desired to quicken the drying operation so as to obtain a harder film in a shorter time, we add a certain amount of boiled linseed oil. In this case, of course, the proportions may also be greatly varied but the following composition has been found to work out extremely well in practice: 27 per cent. pitch, 28 per cent. asphalt, 15 per cent. China wood oil, 10 per cent. cylinder oil and 15 per cent. boiled linseed oil. This constitutes a base which may be thinned for application to cloth by a solvent such as naphtha, benzol, turpentine or the like. The solvent is driven off by baking in a well known manner after the varnish has been applied.

While we have described our invention as embodied in concrete form for purposes of illustration in accordance with the patent statutes, it should be understood that we do not limit our invention thereto, since various modifications thereof will suggest themselves to those skilled in the art without departing from the spirit of our invention, the scope of which is set forth in the annexed claims.

What we claim as new and desire to secure by Letters Patent of the United States, is,

1. A flexible insulating composition comprising China wood oil, pitch and asphalt.

2. A flexible insulating compound comprising China wood oil, pitch, asphalt and a mineral oil.

3. A flexible insulating compound comprising China wood oil, stearin pitch and asphalt.

4. A flexible insulating compound comprising China wood oil, stearin pitch, asphalt and a mineral oil.

5. An insulating compound comprising substantially twenty-five per cent. China wood oil, fifteen per cent. mineral oil, thirty per cent. pitch and thirty per cent. asphalt.

6. A tough, flexible, insulating composition consisting of a mixture of China wood oil, mineral oil, cotton stearin pitch and asphalt.

In witness whereof, we have hereunto set our hands this 11th day of September, 1911.

LAWRENCE E. BARRINGER.  
FRANK C. ZAPF.

Witnesses:

BENJAMIN B. HULL,  
HELEN ORFORD.